

July 1, 1947.

R. T. FIELDS

2,423,182

METHOD OF COLD DRAWING TAPERED FILAMENTS

Filed April 29, 1943

2 Sheets-Sheet 1



*Fig. 2*



*Fig. 1*



*Fig. 3*

*Reuben T. Fields* INVENTOR.

BY *Lynn B. Morris*  
ATTORNEY

July 1, 1947.

R. T. FIELDS

2,423,182

METHOD OF COLD DRAWING TAPERED FILAMENTS

Filed April 29, 1943

2 Sheets-Sheet 2



Fig. 4



Fig. 5

Fig. 7

Reuben T. Fields INVENTOR.

BY *Lynn T. Morris*  
ATTORNEY

## UNITED STATES PATENT OFFICE

2,423,182

## METHOD OF COLD-DRAWING TAPERED FILAMENTS

Reuben T. Fields, Arlington, N. J., assignor to  
E. I. du Pont de Nemours & Company, Wil-  
mington, Del., a corporation of Delaware

Application April 29, 1943, Serial No. 485,925

6 Claims. (Cl. 15—48)

1

This invention pertains to an improved method for making drawn tapered filaments from filaments of cold-drawing-polymeric materials. More particularly, it pertains to an improved method of making flexible tapered bristles from undrawn tapered filaments from orientable synthetic linear polymers. Still more particularly, it pertains to a method of simultaneously making a plurality of tapered bristles from undrawn tapered filaments of orientable synthetic linear polyamides.

An object of this invention is to provide improved tapered filaments which have uniform size, shape, and properties. Another object is to provide tapered filaments in a continuous manner and with uniform results. A further object is to provide a method of cold-drawing tapered filaments which eliminates rupture of such filaments. A still further object is to provide a method of cold-drawing filaments in a continuous manner whereby breakage at the portions of small diameter is eliminated and the portions of larger diameter are adequately drawn. A still further object is to provide a commercially practical method of cold-drawing orientable tapered filaments in multiple whereby the results just indicated may be obtained. A still further object is to provide such a method which requires a minimum of attention by an operator and little maintenance expense. A still further object is to provide a method for making tapered bristles by cold-drawing which utilizes simple and economical machines requiring infrequent mechanical adjustment.

It has been found that tapered filaments of uniform size, shape, and properties can be made by cold-drawing tapered filaments of cold-drawing-polymeric materials, (i. e., solid materials which are capable of being cold-drawn at temperatures below their softening or melting point) between widely separated draw-points at a tension insufficient to cause tensional rupture of the portion of smallest diameter but sufficient to effect drawing of the portions of larger diameter at least to the greater part of the extent to which they are capable of being drawn while heating the filament between draw-points. A moderate temperature insufficient to produce a permanent curl in the filament is desirable. This may be advantageously effected by contact with an aqueous medium at a temperature between 40° and 10° C., and preferably between 50° and 90° C.

In a more limited sense, the invention comprises subjecting a cold-drawing-polymeric organic filament having recurring tapered units

2

uniformly disposed lengthwise therein to cold-drawing between draw-points spaced at a distance not less than five (5) times the unit length (i. e., this distance between successive recurrences of any point in the cycle along the filament) of the drawn tapered filament, at a tension insufficient to cause a tensional rupture of the filament but sufficient to effect a drawing of its portions of larger diameter to at least 80% of the extent to which they are capable of being drawn at a speed so that the travel of a given fixed point in the filament requires at least two (2) seconds to pass from the first to the second draw-point while contacting the filament between draw-points with an aqueous medium at a temperature from 50 to 90° C. for a period of at least one (1) second.

The invention in its preferred aspect is concerned with the cold-drawing of orientable organic filaments having tapered units uniformly disposed lengthwise therein, to tapered filaments suitable for cutting into bristles for paint and like brushes wherein the maximum diameters of the tapered bristles are not less than 0.008" and not greater than that which will result in a flexible, supple brush and especially with such bristles composed of synthetic linear polyamides. After the cold-drawing operation, the tapered filaments may be further conditioned and/or cut at the thick and/or thin portions and assembled.

The invention, as specifically applied to the cold-drawing of tapered filaments in multiple, comprises the further step, preliminary to the drawing itself, of arranging the several filaments of a group side by side in a single plane and, preferably, close together and to that end provides in advance of the drawing equipment itself means for thus bringing together the several filaments into a ribbon-like arrangement. Conveniently, this means takes the form of a flat or slightly concave guide interposed between the normal straight line of travel of the filament. The means may advantageously also deflect the filament from the line of travel, for instance, about 20 to 60°.

The invention will be more readily understood by the following detailed description with reference to the accompanying drawings but it is to be understood that the description is given by way of example only and is in no respect limitative. In the drawings similar reference numerals refer to similar parts throughout the several views:

Figure 1 is a view in side elevation of a suit-

able form of apparatus for carrying out the invention;

Figure 2 is a view in plan of the same apparatus;

Figure 3 is a view in elevation of part of the equipment taken along the line 3-3 of Figure 1;

Figure 4 is an enlarged view in elevation of the drawing rolls showing the line of path of the filaments;

Figure 5 is a plan view of the drawing rolls of Figure 4;

Figure 6 is an enlarged view of the guiding means shown in Figures 4 and 5, and

Figure 7 is a sectional view along the line 7-7 of Figure 6.

The drawing of the filament is accomplished by the difference in peripheral speeds between two pairs of drawing rolls, of which the pair 11 and 12 are the low speed rolls and the pair 13 and 14 are the high speed rolls. The rolls 11 and 12 are driven from a shaft 15 through spiral gears 16 and 17. The rolls 13 and 14 are similarly driven from the shaft 18 by spiral gears 19 and 20. The shaft 15 is driven by the shaft 16 through sprockets 21 and 22, and thus the relative speeds of the two shafts are subject to control according to the selection of the sprockets 21 and 22. The speeds of rotation of the pairs of rolls 11, 12 and 13, 14 are further variable by selection of the respective spiral gears 16, 17 and 19, 20. The peripheral speeds of rolls 11 and 12 are the same, and the peripheral speeds of rolls 13 and 14 are the same. The ratio of the peripheral speed of the pair of rolls 13, 14 to that of the pair of rolls 11, 12 governs the amount of stress imposed upon the filament during the operation of drawing. If, for example, the peripheral speed of the faster rolls is four times the peripheral speed of the slower rolls, then the "draw ratio" is, theoretically, 4:1, and the initial length of the filament is increased by 300 per cent during the drawing. Actually, however, because of the occurrence of some elastic recovery after the tension has been removed, the permanent stretch will usually be somewhat less than 300 per cent, and the actual draw ratio somewhat less than 4:1, e. g., 3.7:1.

In actual construction, the pair of rolls 11, 12 may be placed, for convenience, directly above the pair 13, 14. However, in order the better to diagram the course of the filament through the equipment, the rolls 13, 14 are shown mounted upon longer shafts than is actually the case, so that they project apparently into a position which is not directly beneath the other rolls, and correspondingly the alignment of parts 21, 24 and 25 in the horizontal is distorted in the figures.

As is clearly indicated in Figure 3, the axes of the rolls 11 and 12 are not parallel, the one tilting slightly below the horizontal and the other slightly above the horizontal. The actual angle between these positions should be of the order of about ten degrees, but is exaggerated in the figures for the sake of clearness. The purpose of this tilting of the axes is to cause each of these rolls 11 and 12 to serve as a spreader for the other. Similarly, the axes of rolls 13 and 14 are not parallel to each other, but the angle between these rolls needs to be only about one-half as great as that between the rolls 11 and 12, because the ribbon of drawn filaments which is handled by 13, 14 is only approximately half as wide as the ribbon of undrawn filaments handled by 11, 12, and hence a smaller advance by spreading action is sufficient to space the successive wraps.

The filament 23 having tapered portions coming from a spool or directly from the preceding operation enters the system from the left in Figures 1 and 2 and is wrapped several times around the pair of rolls 11, 12, as indicated in Figures 2 and 3. The fact that these two rolls are not parallel causes each one to serve to advance the position of successive turns of the filament upon the other. After its last turn around these rolls, the filament 23 passes from the upper face of the roll 11 to an idler roll 24 several feet distant, and thence back to the lower face of the roll 14, and passes several times around the pair of rolls 13, 14 in the manner described in connection with rolls 11, 12. After its last turn around this pair of rolls 13, 14, the filament passes to a wind-up spool 25.

The system is driven by a motor 26 by way of a countershaft 27. Through sprockets 28 and 29 this countershaft 27 drives the shaft 18 to operate the two pairs of rolls 11, 12 and 13, 14. Through bevel gears 30 and a countershaft 31 the countershaft 27 drives a shaft 32 to operate the windup spool 25. The shaft 32 drives the spool 25 by way of a multiplate clutch 33, the slipping of which permits of the maintenance of a constant peripheral speed as the effective diameter of the spool 25 becomes increased by the filament wound upon it. It is desirable to provide a traverse mechanism by which the filament is guided to the spool 25 so as to form orderly layers thereupon, but this mechanism constitutes no part of the present invention and is omitted from the drawing for purposes of simplification.

The essential moving parts of the drawing equipment proper are the two pairs of rolls 11, 12 and 13, 14. The traction resulting from the several wraps of the filament around each of these pairs of rolls makes each pair serve as one of the points of application of the tension which results from the difference in peripheral speeds of the two pairs. These points of application of tension, or more briefly, "draw-points," are separated, in accordance with the invention, by a distance which is large compared with that of the prior art. This long span of filament between draw-points may be provided by installing the two pairs of rolls at a corresponding distance from each other, but the same result is accomplished by the arrangement already described, and illustrated in Figures 1 and 2, in which the span of filament between the two pairs of rolls is made as long as desirable by the interposition of a remotely placed idler, 24, while the rolls themselves are kept in actual proximity to each other for the sake of making the equipment more compact and the driving mechanism more simple.

The long span between draw-points is an important feature of the invention and has numerous advantages. It reduces the risk of breakage of the filament which is undergoing elongation during its passage between draw-points, even though the magnitudes of the tension and the draw ratio are unchanged by the wide separation.

When the tapered filament is passed continuously between draw-points its portions of smallest diameter are generally the first to be elongated by the tension. They seem to be drawn immediately upon entering the span between the draw-points. Moreover the portions of largest diameter also become drawn to some extent.

The further drawing of the portions of largest diameter without tensional failure is accomplished as stated above by heating the filament between draw-points to a moderate temperature,

e. g., between 40 and 100° C. In the preferred aspect of the invention this is effected by contact with a heated aqueous solution. However the heating may be done by utilizing heated fluids which are inert toward the filaments. Heated gases or vapors such as air, nitrogen, steam, may thus be used. Similarly other inert liquids such as aliphatic and aromatic hydrocarbons which are liquids at the temperatures may be used. A liquid medium is generally more effective because of its greater heat capacity.

Heating of the filament by contact with an aqueous liquid, e. g. hot water, is very simply accomplished by placing in the line of travel of the filament 23, as shown in Figs. 1 and 2, an open-ended trough 37 into which hot water is continuously fed through an intake 38 and from which it drains away at the other end through an outlet 39.

The beneficial effect of heating the filaments by contact with hot water between draw-points in accordance with the invention is particularly marked with polyamides such as hexamethylene sebacamide. The tension required to draw such a filament at about room temperature is reduced by about 27% by changing the temperature from 27° C. to 82° C. while the tensile strength is reduced only 4%. In the case of hexamethylene adipamide, a similar reduction occurs, the tension being reduced about 20% while the tensile strength is reduced to a significantly less degree.

The drawing in general is effected so that the filament is elongated in a ratio between 3.6 to 1 and 4 to 1. While this will not in all cases result in a complete drawing of the portions of greatest diameter, it is usually sufficient for tapered bristles for paint brushes and the like because the portions of smaller diameter are fully drawn. The large ends of the bristles are contained at least in part within the grip of the brush where a slight proportion of incompletely drawn filament is not a serious defect.

The foregoing details of drawing technique are applicable to a single tapered filament or a group of tapered filaments. For commercial operations, it is preferable to simultaneously draw a plurality of filaments. This may be advantageously done by arranging a plurality of them in a ribbon-like group, i. e. parallel in the same plane and preferably each in contact with its neighbor during the entire operation. This can be accomplished through the use of guides. For instance a guide of rigid material (e. g. metal, glass, plastic, ceramic, etc.) which presents a straight or slightly concave contour in a plane at right angles to the filament is interposed across the line of filaments coming from a previous operation or from storage spools, in such a position as to cause the bundle of filaments to change its path by an appreciable angle preferably 20 to 60 degrees. Such a device is shown in Figs. 4 and 5 in cooperation with the roll 11 described above. A large scale is used to show the unit structure of the filaments (which is somewhat exaggerated) action of the guide and entry of the ribbon-like groups into the drawing equipment proper. Only a few tapered units are shown in order to avoid confusion. In actual practice the tapered units may be close together and have various contours. The tapers may be steep, gradual, curved or have relatively flat portions at the points of maximum or minimum diameter. Suitable methods for preparing the undrawn tapered filaments with re-

curring units are described in U. S. P. 2,292,905 and, more particularly, in Alftan and Fields U. S. P. 2,418,492.

In Figures 4 and 5 the individual filaments are shown as being in phase, i. e., the points of maximum and minimum diameter are together. This condition, while not absolutely essential to its success, is highly desirable and enables a bundle of the drawn tapered filaments to be cut by automatic means in a subsequent operation. If the filaments are delivered to the guide 34 and first drawing roll in phase they ordinarily will continue in that manner throughout the drawing operation.

15 The guide 34 may take other forms than the specific one shown. For example, a roller of concave contour may be used. The roller or stationary guides may further be provided with grooves corresponding to the desired positions of the several filaments. In fact, the prolonged usage especially of a stationary guide will develop grooves as a result of abrasion by the filaments.

20 If the bundle of tapered filaments being fed to the drawing equipment is in non-contact, as is the group 23 of three filaments, shown in Figures 4 and 5, the desired arranging of them into a ribbon-like group is readily accomplished, as indicated in Figure 6, by use of the operator's finger 38 or finger and thumb. The arrangement, once 25 established in this simple manner, is maintained indefinitely by the action of the guide 34 so long as the filaments of the group approaching it are not actually twisted around each other. The concavity of the face of the guide causes the several 30 filaments to lie closely side by side, in actual contact at each recurrence of the maximum diameter of the filament.

35 The frictional resistance of the passage of the filaments over the guide, is reduced by having the filament approach the guide in wet condition. This is readily achieved by having the filament pass through a container of water en route to the guide. Furthermore, the presence of a film of water upon the filaments is conducive to maintaining the several filaments of the ribbon-like 40 group in contact with its neighbor.

The arrangement of the filaments side by side, in phase, and in contact offers convenience in 45 making an accurate measurement of the maximum diameter of the filament, for purposes of control, by measuring the total width of the ribbon and dividing by the number of filaments which it contains.

50 But the principal purpose and advantage of arranging the plurality of filaments in phase in a single plane before drawing is that it ensures exactly equal treatment of each individual filament in the drawing operation. This is important in order to prevent the group from getting out of 55 phase, and also because it eliminates frictional effects between filaments in contact which, in the case of a random bundle of filaments subjected to drawing, are likely to cause weakening or breakage of one filament by the rubbing action of its 60 neighbor.

65 Figures 4 and 5 show also, on an enlarged scale, the passage of the filament 23 to, around and from the slow speed rolls 11 and 12 of the drawing equipment already described. It will be observed that the spreader action of these two rolls causes the ribbon-like group of filaments 23 to progress from the rear to the front of this pair of rolls in its successive passages around them. It is to be noted also that the filament 70 when once relieved of the tractive anchorage and

subjected to tension in the beginning of its passage from its last wrap around roll 11 across the span to the high speed rolls begins immediately to undergo stretching, i. e., cold-drawing, in its portions of smallest diameter, as evidenced by the greater difference between successive points of maximum diameter in the filament at this stage (a'-b') than prior to the beginning of the drawing (a-b).

The invention provides a practicable, inexpensive, and effective method of cold-drawing, on a commercial scale, undrawn tapered filaments. In its preferred embodiment, involving drawing a plurality of filaments while side by side in a single plane, it subjects all of the individual filaments of a multiple group to the same drawing treatment and thus maintains in phase a group of filaments delivered to the drawing equipment in phase. Moreover, it delivers the drawn filament still in phase to subsequent operations, e. g., conditioning and cutting.

The equipment required for the process of the invention is simple, requires no close supervision, and can be readily maintained in operating condition. The rolls between which the drawing tension is applied may be made of generous size and correspondingly sturdy. Their faces may be made of metal or other durable material, whereas the previously proposed machines have small rolls coated with rubber, or the like, which require frequent inspection and adjustment and need replacement or repair.

The recognition, in accordance with the invention, of the lack of need of completeness of drawing of the coarser portions of tapered filaments which are to serve as the butts of individual pieces used as "bristles" in paintbrushes, and the like, extends the utility of the invention to the cold-drawing of certain tapered filaments which by reason of their material and/or their dimensions can not, even by the process of the invention, be fully drawn in their coarser portions without breakage of their finer portions, and also provides a factor of safety in the handling of tapered filaments which are not subject to this difficulty.

It will be evident that the invention, with respect to the drawing technique itself, has its chief value in connection with the drawing of tapered filaments of which the unit length is short, e. g., filament to be used in paintbrushes but is also useful for tapered film. In the case of tapered filament of great unit length, such as is used as fishing leaders, the method of Smith, U. S. P. 2,292,905, which limits the distance between draw-points, becomes commercially feasible, even without the use of rubber rolls to fix the draw-points. But the guide provided by the present invention as a means of maintaining a plurality of filaments in a ribbon-like group will be useful in connection with Smith's technique as applied to fishing leader filament.

The invention will obviously be applicable to tapered filaments of materials other than those mentioned herein so far as they are similar thereto in significant properties.

The invention is not limited to the preparation of tapered filaments or bristles from the two specific polyamide filaments given above. On the contrary, it may be applied to any tapered filament which can be cold-drawn. The preferred polymeric filaments are polyamides of the types described in U. S. Patents 2,071,250, 2,071,253, and 2,130,948. These polyamides are prepared from bifunctional polyamide-forming reactants and

contain amide groups as an integral part of the main chain of atoms in the polymer. It is not essential that the linking group in the polymer chain consist solely of amide groups; they may also contain other groups, e. g. ester groups.

The polyamides are of two general types, those derived from diamines and suitable dicarboxylic acids or amide-forming derivatives of dibasic carboxylic acid, and those derived from polymerizable amino acids or amide-forming derivatives thereof, e. g. esters and lactams. On hydrolysis with hydrochloric acid the polyamides yield polyamide-forming reactants; polyamides of the diamine-dibasic acid type yield a diamine hydrochloride and a dibasic carboxylic acid, whereas those of the amino acid type yield an amino acid hydrochloride. As specific examples of such polyamides may be mentioned polydecamethylene adipamide, polyhexamethylene sebacamide, poly-pentamethylene sebacamide, polyoctamethylene adipamide, 6-aminocaproic acid polymer, and 11-aminoundecanoic acid polymer. Mixtures of polyamides and interpolyamides may also be used. Examples of such interpolyamides are those derived from hexamethylenediamine, decamethylenediamine, adipic acid and sebacic acid, and from hexamethylenediamide, adipic acid, and 6-aminocaproic acid. As examples of polyamides containing groupings other than amide-groupings may be mentioned ester-amide interpolymers, such as may be derived from a diamine, a dibasic acid, and a glycol or from an amino acid and an hydroxy acid. For paint brushes preferred materials will include the superpolyamide hexamethylene sebacamide or hexamethylene adipamide alone or in admixture with 2% to 30%, and especially about 10%, of phenolformaldehyde resin. Such materials are described in assignee's application Serial No. 397,887.

40 The term "polyamide" as used in this application includes polymers containing a plurality of groups of structure



45 regardless of the nature of the atom to which the indicated free linkages are attached. The term includes polymers derived from a glycol and a diisocyanate or a diisothiocyanate.

50 The tapered filaments of this invention need not necessarily consist wholly of polyamide or modified polyamide. It is frequently desired to deluster and/or color the filaments by adding a pigment to the polymer or to the reactants from which the polymer is prepared. It is also useful in many cases to dye the filament, for example with nigrosine black, Sudan brown, etc. Thus, fishing lines or leaders may be made to resemble closely water of almost any color or turbidity by the proper choice of dyes or pigments. Bristles may also be made of any desired color and length. For paint brushes a unit length of 4 to 18 inches is practical.

55 It will be evident that the invention has its chief value in connection with the drawing of tapered filaments of which the unit length is short, e. g., a filament useful in paint brushes, and the like, but is also useful for longer tapered filaments, e. g., fishing leaders.

60 As many apparently widely different embodiments of this invention may be made without departing from the spirit and scope thereof, it is to be understood that the invention is not limited to the specified embodiments thereof except as defined in the appended claims.

I claim:

1. The process which comprises subjecting a cold-drawing organic polymeric filament having recurring tapered units uniformly disposed lengthwise, while passing between draw-points spaced at a distance at least five times the length of a tapered unit in drawn condition, to tension and heating the filament between such points to a temperature of approximately 40° C.-100° C.

2. The process which comprises subjecting a cold-drawing organic polymeric filament having recurring tapered units uniformly disposed lengthwise, while passing between draw-points spaced at a distance at least five times the length of a tapered unit in drawn condition to a tension insufficient to cause tensional failure of the filament but sufficient to effect drawing of the portions of larger diameter to at least 80% of the extent to which they are capable of being drawn and heating the filament to a temperature from 50° and 90° C. between such points.

3. The process which comprises subjecting a cold-drawing organic polymeric filament having recurring tapered units uniformly disposed lengthwise, while passing between draw-points spaced a distance such that the travel of a fixed point of the filament requires at least two seconds and at least five times the length of a tapered unit in drawn condition, to a tension insufficient to cause tensional failure of the filament but sufficient to effect drawing of the portions of larger diameter to at least 80% of the extent to which they are capable of being drawn, and heating the filament between such points by contacting it with water at a temperature between 50° and 90° C.

4. The process which comprises subjecting a filament composed of a synthetic linear polyamide capable of being cold-drawn having recurring tapered units of short unit length uniformly disposed lengthwise, while passing between draw-points spaced a distance such that the travel of a fixed point of the filament requires at least two seconds and at least five times the length of a tapered unit in drawn condition, to a tension insufficient to cause tensional failure of the filament but sufficient to effect drawing of the portions of larger diameter to at least 80% of the extent to which they are capable of being drawn and heating the filament between such points by contacting it with water at a temperature between 50° and 90° C. for a period of at least one second.

5. The process which comprises subjecting a cold-drawing polyhexamethylene sebacamide filament having recurring tapered units uniformly disposed lengthwise, while passing between draw-points spaced a distance at least five times the length of a tapered unit in drawn condition, to a tension insufficient to cause tensional failure of the filament but sufficient to effect drawing of the portions of larger diameter to at least 80% of the extent to which they are capable of being drawn and heating the filament to a temperature from 50° and 90° C. between such points.

6. The process which comprises subjecting a filament composed of polyhexamethylene sebacamide and having recurring tapered units of short unit length uniformly disposed lengthwise, while passing between draw-points spaced a distance such that the travel of a fixed point of the filament requires at least two seconds and at least five times the length of a tapered unit in drawn condition, to a tension insufficient to cause tensional failure of the filament but sufficient to effect drawing of the portions of larger diameter to at least 80% of the extent to which they are capable of being drawn and heating the filament between such points by contacting it with water at a temperature between 50° and 90° C. for a period of at least one second.

REUBEN T. FIELDS.

#### REFERENCES CITED

The following references are of record in the file of this patent:

#### UNITED STATES PATENTS

| Number       | Name             | Date           |
|--------------|------------------|----------------|
| 2,321,635    | Taylor           | June 15, 1943  |
| 2,142,912    | Moncrieff et al. | July 3, 1939   |
| 2,217,707    | Samerdyke et al. | Oct. 15, 1940  |
| 40 2,234,540 | Fryer            | Mar. 11, 1941  |
| 2,292,905    | Smith            | Aug. 11, 1942  |
| 1,878,692    | Furness          | Sept. 20, 1932 |
| 936,243      | Frappier         | Oct. 5, 1909   |
| 2,199,411    | Lewis            | May 7, 1940    |
| 45 2,293,825 | Hosfield         | Aug. 25, 1942  |
| 2,137,235    | Carothers        | Nov. 22, 1938  |

#### FOREIGN PATENTS

| Number     | Country       | Date          |
|------------|---------------|---------------|
| 50 541,261 | Great Britain | Nov. 19, 1941 |
| 50,332     | France        | Dec. 1, 1939  |

Addition to Patent No. 833,756

**Certificate of Correction**

Patent No. 2,423,182.

July 1, 1947.

**REUBEN T. FIELDS**

It is hereby certified that errors appear in the printed specification of the above numbered patent requiring correction as follows: Column 2, line 37, for "iself" read *itself*; column 5, line 73, for "or or" read *or*; column 6, line 42, for "an" before "route" read *en*; column 8, line 74, for "specified" read *specific*; and that the said Letters Patent should be read with these corrections therein that the same may conform to the record of the case in the Patent Office.

Signed and sealed this 2nd day of September, A. D. 1947.

[SEAL]

**LESLIE FRAZER,**  
*First Assistant Commissioner of Patents.*